

Jan. 17, 1939.

L. B. CARRIZO

2,144,328

# PROCESS FOR TREATING AND PURIFYING SODIUM CHLORIDE

Filed Dec. 2, 1935

2 Sheets-Sheet 1



Inventor:  
Luis Bartolome Carrizo.  
By Brown, Jackson, Portchell and Dickey  
Attys.

Jan. 17, 1939.

L. B. CARRIZO

2,144,328

PROCESS FOR TREATING AND PURIFYING SODIUM CHLORIDE

Filed Dec. 2, 1935

2 Sheets-Sheet 2



Inventor:  
Luis Bartolome Carrizo  
By Brown, Jackson, Botteler, Newman  
Atty's

## UNITED STATES PATENT OFFICE

2,144,328

PROCESS FOR TREATING AND PURIFYING  
SODIUM CHLORIDE

Luis Bartolomé Carrizo, Quilino, Argentina

Application December 2, 1935, Serial No. 52,519½

4 Claims. (Cl. 209—2)

The present invention relates to a process for purifying salt or sodium chloride, whereby it is possible to free this substance of the impurities contained therein, for the purpose of rendering it suitable for consumption.

It is known that certain impurities commonly found in salt in its natural state, particularly the magnesium compounds, readily absorb moisture and, when heated, conglomerate in the form of pellets. The process according to the present invention is based upon this hygroscopic quality inherent in said impurities, with the end in view of purifying the sodium chloride. The process may be performed by a special arrangement or means of comparatively simple construction and operation.

By way of example, the attached drawings show apparatus of a type suitable for practicing the process of this invention.

20 In the drawings:

Figure 1 is a front view of a set of kilns and a sifter used in practicing the process of my invention;

25 Figure 2 is a sectional view taken substantially on line A—B of Figure 1;

Figure 3 is a side view of the sifter, on an enlarged scale;

Figure 4 is a front view of the sifter shown in Figure 3;

30 Figure 5 is a plan view of the kilns and sifter shown in Figure 1;

Figure 6 is a longitudinal sectional view, on an enlarged scale, of the body of the sifter; and

35 Figure 7 is a sectional view taken substantially on line C—D of Figure 6.

In the different figures of the drawings, the same reference numbers indicate the same parts.

The illustrated arrangement or apparatus for practicing the process of my invention comprises 40 two similar kilns 1. These kilns are preferably formed of brickwork of fireproof material.

Each kiln 1 is composed of a furnace 2 and an ash pit 3 provided with openings 2' and 3' for feeding the kiln and discharging the ashes, respectively. These openings, which may be fitted with suitable doors, provide for internal air draught.

As may be observed in Figure 2, a horizontal partition 5 is arranged within the furnace 2 having passage 6 at the back thereof, through which the hot gases and the combustion smoke are conducted. Passage 6 opens at its upper end into a space or hot chamber 7, between partition 5 and the top wall of the kiln, into which space opens 55 a stack 8 for creating a draft through furnace 2 and space 7, this stack discharging into the atmosphere. On top of the kiln 1 there is a heating surface 9 surrounded by a low railing or retaining wall 10.

60 Between kilns 1 a space is left, as may be seen

in Figures 1 and 5, which space accommodates the sifting machine, illustrated more fully in Figures 3, 4, 6 and 7.

The sifting machine comprises a hopper 11 from which troughs 12 extend upward to the tops of the kilns 1, adjacent the heating surfaces 9 thereof. Hopper 11 is arranged on a scaffold 13 and communicates with the upper end of a casing mounted on the scaffold at an inclination downward and forward thereof, by means of 10 flexible rods 15.

For the purpose of imparting a reciprocating motion to casing 14, I provide a shaft 16 on which is secured an eccentric 17 connected by a rod 18 to casing 14 beneath the latter. Shaft 16 is journaled in suitable bearings on the scaffold 13 and is provided at one end with a pair of pulleys 19 and 20, one being fast to the shaft and the other loose thereon, adapted to be driven through an endless belt in connection with a motor (not 20 shown), providing a drive of known type. Any other suitable means may be provided for rotating shaft 16 by means of a motor, or rotary movement may be imparted to the shaft by hand power, by arranging a crank on one end of the 25 shaft, in a known manner which need not be illustrated.

Within the casing 14 (see Figure 6) there are conveniently arranged a coarse mesh sieve 21 and a fine mesh sieve 22, the latter being placed beneath sieve 21. If desired, additional sieves of 30 increasingly finer mesh downward, in accordance with the different degrees of fineness of salt it is desired to obtain, may be provided, as will be readily understood from the following explanation, and which need not be illustrated.

The sieves 21 and 22 divide the casing 14 into three compartments or chambers having at the front thereof, respectively, outlets 23, 24 and 25, the first outlet 23 being for the impurities commonly termed "tailings", the second outlet 24 being for the sodium chloride in small lumps, and the third outlet 25 being for sodium chloride in finely powdered form.

The process in accordance with this invention 45 is as follows:

The crude salt which is extracted from the salines, is first passed through a grinding mill of known type. If the salt is already available in a more or less divided state, grinding may be dispensed with.

In order to expel the moisture and cause the formation of the conglomerates of the impurities contained in the sodium chloride, the crude salt, which has previously been ground, when necessary, is applied to the heating surfaces 9 of the kilns 1, which surfaces are suitably heated, striving to hold their temperature between 80° and 100° centigrade.

By spreading the salt upon the surfaces 9 and 60

agitating it by means of a rate or any other suitable tool, the water contained therein will be expelled by evaporation, while simultaneously the impurities will absorb a portion of the water and form pellets, by virtue of their hygroscopic character referred to thus forming the tailings. When this operation has been completed, the salt is transferred, conveniently by means of the rakes or other tools, to the troughs 12, and by, the latter, 10 to the hopper 11, whence it passes into the casing 14 onto sieve 21.

15 The impurities or tailings which, on account of their conglomeration, will not pass through the sieve 21, are discharged through the outlet 23, whereas the particles of sodium chloride readily 20 pass through said sieve 21 and fall upon the sieve 22, which is of fine mesh. The more or less coarse grained salt will be discharged through outlet 24, while the salt in finely powdered form, which 25 passes through the fine mesh sieve 22, will be discharged through outlet 25. In order to facilitate the movement of the salt and prevent clogging of the sifter, the casing 14 is reciprocated in the manner previously described.

25 At the respective outlets 23, 24, and 25, suitable containers may be provided for collecting the materials issuing therefrom. The tailings discharged from outlet 23 may be rejected, and the sodium chloride discharged from outlets 24 and 30 25 may be suitably packed for transportation and sale.

35 The sodium chloride is thus collected in almost a chemically pure state, the originally contained impurities having been effectively separated therefrom by the combined action of heating and agitation, with accompanying conglomeration of the impurities, during the drying process to which the crude salt extracted from the mines is subjected.

40 In the following is given, by way of illustration only, an analysis of 100 grams crude salt extracted from "Salinas Grandes" (Province of Cordoba, Argentine Republic) in order to establish the ingredients forming conglomerations and the quantity of sodium chloride which is obtained:

100 grams crude salt, dried, contains

|                                                    | Grams    |
|----------------------------------------------------|----------|
| Water                                              | 0.00000  |
| Insoluble inorganic matters                        | 0.05760  |
| Insoluble organic matters                          | 0.4011   |
| Calcium sulphate (CaSO <sub>4</sub> )              | 0.09977  |
| Magnesium sulphate (MgSO <sub>4</sub> )            | 0.00452  |
| Sodium sulphate (Na <sub>2</sub> SO <sub>4</sub> ) | 0.47592  |
| Sodium chloride (NaCl)                             | 99.31242 |
| Nondetermined matter                               | 0.00925  |
|                                                    | 99.99959 |

Such substances as are foreign to the sodium 60 chloride will almost entirely conglomerate during the drying and agitating treatment on the

kilns 4, forming pellets which are easily separated in the sifting operation, in such manner as to obtain the sodium chloride in a pure state, the particles of foreign substances which succeed in getting past the sieves and mixing with the salt 5 proper forming an infinitesimal quantity which may be disregarded.

Modifications may be introduced without departing from the scope of the present invention, as defined in the appended claims. 10

I claim:

1. The process of treating a mixture of sodium chloride and hygroscopic impurities for removal of the latter from the sodium chloride, which comprises heating the mixture to a maximum temperature of approximately 100° C. and drying the sodium chloride by the combined action of heat and absorption of moisture by the hygroscopic impurities while conglomeration the latter in the form of pellets, and separating the dried sodium 15 chloride from the pellets of conglomeration impurities.

2. The process of treating a mixture of sodium chloride and hygroscopic impurities for removal of the latter from the sodium chloride, which comprises spreading the mixture in a relatively thin layer upon a heating surface, there heating the mixture to approximately 80° C. while stirring it, thereby drying the sodium chloride by the combined action of heat and absorption of moisture by the hygroscopic 25 impurities while conglomeration the latter in the form of pellets, and separating the dried sodium chloride from the pellets of conglomeration impurities.

3. The process of treating a mixture of sodium chloride and hygroscopic impurities for removal of the latter from the sodium chloride, which comprises spreading the mixture in a relatively thin layer upon a heating surface, there heating the mixture to a temperature of approximately 30 100° C. while stirring it, thereby drying the sodium chloride by the combined action of heat and absorption of moisture by the hygroscopic impurities while conglomeration the latter in the form of pellets, and separating the dried sodium 45 chloride from the pellets of conglomeration impurities.

4. The process of treating a mixture of sodium chloride and hygroscopic impurities for removal of the latter from the sodium chloride, which comprises spreading the mixture in a relatively thin 50 layer upon a heating surface, there heating the mixture to a temperature between approximately 80° and 100° C. while stirring it, thereby drying the sodium chloride by the combined action of heat and absorption of moisture by the hygroscopic impurities while conglomeration the latter in the form of pellets, and separating the dried sodium chloride from the pellets of conglomeration 55 impurities.

60 LUIS BARTOLOMÉ CARRIZO.